

# United States Patent Office

3,075,228

Patented Jan. 29, 1963

1

3,075,228

ANTI-FOGGING ARTICLE  
Nathaniel M. Elias, 56 Washington Mews,  
New York, N.Y.

No Drawing. Filed Feb. 24, 1958, Ser. No. 716,848  
19 Claims. (Cl. 15—506)

The present invention relates to a new article of manufacture adaptable for cleaning and treating smooth glass-like surfaces, a process of making the article and a method of treating glass, plastic or polished surfaces therewith.

This is a continuation-in-part of application Serial No. 354,432, now abandoned.

It has been suggested in the prior art that fibrous material be impregnated with certain sulfated aliphatic hydrocarbons for the purpose of providing an article which may be used for polishing and inhibiting fog formation on glass and the like. Polyhydroxy alcohols that have been partially esterified with higher fatty acids have also been suggested for somewhat similar purposes. These materials, however, exhibit certain disadvantages which have limited their usefulness. Thus, these agents are held too tenaciously in the fibrous materials, so that there is difficulty in transferring them to the glass surface. It has now been found that these disadvantages may be overcome through the use of a composition comprising at least one salt of sulfated alkyl aryloxy polyalkoxy alcohol. It has further been found that the feel of the impregnated fibrous material is considerably improved through the use of said composition.

In accordance with the present invention fibrous material is impregnated with a composition containing at least one compound of formula

(1)



wherein  $n$  is an integer preferably from 8 to 100; R is an alkyl radical, and preferably higher alkyl radical; R' is a divalent saturated alkylene radical having at least 2 carbon atoms preferably lower alkylene; Me is a metal or metalloid cation, and preferably alkali metal. R may be an alkyl radical having from 1 to 30 carbon atoms and preferably from 8 to 32 carbon atoms. Thus, R may be methyl, ethyl, n-propyl, isopropyl, n-butyl, t-butyl, pentyl, hexyl, 2-ethylhexyl, octyl, nonyl, decyl, hendecyl, do-decyl, tridecyl, tetradecyl, pentadecyl, eicosyl and dotriacontyl. R' may be a divalent saturated alkylene radical having preferably from 2 to 3 carbon atoms and including ethylene and propylene, or mixtures of both in the polyglycol chain. Me in Formula 1 above may be an alkali metal, such as sodium, potassium or lithium. The best results are obtained with compounds wherein R is octyl, or nonyl; R' is ethylene, i.e.,  $-\text{CH}_2\text{CH}_2-$ ; and Me is sodium. In the preferred form of this invention the groups bonded to the benzene ring in Formula 1 are in the para position to each other.

It has been found, in accordance with certain features, of the present invention, that the combination of a substantial percentage of a compound of Formula 1, which is solid at room temperature, and a flexible web-like fabric such as paper, felt and textile, produces an article highly useful for cleaning and defogging glass surfaces. The compounds are solid in the ordinary temperature range between 15° and 45° C., and are water soluble. The solubility is sufficient so that a trace of moisture, such as is usually present as an adsorbed film on glass or plastic surfaces, is sufficient to dissolve a minute amount of said compounds from the cloth and leave it as an invisible film on the glass surface.

The compounds of Formula 1 do not easily form insoluble precipitates or residues with impurities generally present in water—such as calcium, iron, etc. Nor is the

2

trace of material left on the glass or transparent plastic which may be only one or two microns thick, opaque or interfere with the passage of light.

It has been found, in accordance with the present invention, that unexpectedly, large amounts of the compounds of Formula 1, based on the weight of the fabric, can be incorporated into such fabric and will adhere and remain part of the resulting article. Moreover, the fabric will remain flexible, will be changed very little in appearance, and will be usable over a long period of time. Furthermore, it has been found that said compounds are readily transferred to the glass surface.

The proportion of Compound 1 described above which may be incorporated into a fabric to make it useful for the purposes of the present invention, may range from a low of about 3% of the original weight of the fabric up to 100% or even more. I have found that proportions less than 3% based on the original weight of the textile are not effective because the textile retains such material by adsorption and does not release it to the glass or other surface early enough to be properly effective.

In accordance with the present invention, any salt of a sulfated alkyl aryloxy polyalkoxy alcohol, as defined herein, or any mixture of such compounds, may be advantageously employed. Thus, for example, the sodium salts of sulfated octylphenoxy-polyethoxy ethanol or sulfated nonylphenoxy-polyethoxy ethanol, either individually or in admixture, are excellent fogproofing agents.

It has also been found that in some cases, in addition to the compounds of Formula 1 above, it is desirable to add a small proportion of a nonionic wetting agent. Among the nonionic wetting agents that may be mentioned are the mono methyl, ethyl, propyl or decyl ethers of high molecular weight polyglycols. Similarly monoesters of polyglycols may be added. These include, for example, polyethylene or polypropylene glycol-monolaurate, -mono oleate, -mono stearate, -mono ricinoleate, etc. For additional nonionic wetting agents that are useful in the present invention, see "Surface Active Agents" by Schwartz & Perry, pages 202-214. In contrast to this, the cationic surface active agents are definitely useless for antifogging, since they actually promote fogging on glass or plastic.

It has also been found that in combination with the compounds of Formula 1 a useful composition includes a small quantity of a sodium alkyl sulfate, such as sodium lauryl sulfate. In a similar manner, other anionic materials in small quantities may be used in conjunction with compounds of Formula 1. These include the alkali salts of naphthyl sulfate, e.g., the sodium sulfonate of polypropyl naphthalene (sold under the trade names of Akanol B, Nekol A, etc.). These are examples of the aralkylsulfates that may be used in conjunction with the compounds of Formula 1. The sodium salt of keryl-benzene sulfonate (sold under the trade names of Nacconal NRSF, etc.), may similarly be used.

When the principal antifogging agent is used in conjunction with the secondary agents, such as the nonionic wetting agents, the ratio of the principal antifogging agent to the secondary agents are employed in the range of 85 to 15 parts by weight of secondary agent per part of principal agent and preferably 75 to 25 parts by weight of secondary agent per part of principal agent.

The articles of the present invention may be made from a large variety of fibrous materials. These include knitted, woven fabrics of cotton, wool, linen, rayon, etc. as well as conglomerate masses of fibers of these and similar materials. They may also be prepared from synthetic fiber cloth.

The following examples are further illustrative of the present invention. However, the invention is not restricted thereto. The sodium salt of the sulfated octyl-

## 3

phenoxyethoxy ethanol of the examples below is prepared by the sulfation and neutralization with sodium hydroxide of octyl phenoxyethoxyethanol prepared by the reaction of 9 moles of ethyleneoxide with 1 mole of p-octylphenol. The monomethyl ether of polyglycol mentioned in the examples is prepared by the reaction of 1 mole of a methylhalide with 1 mole of monosodium polyethylene glycolate of molecular weight 400. The sodium salt of the sulfated nonyl phenoxyethoxyethanol employed in the following examples is prepared in the same way as the octyl compound except that 10 moles of ethylene oxide are reacted with 1 mole of p-nonylphenol, the product then being sulfated and neutralized. Unless otherwise specified, the percentages given are by weight.

## Example 1

A 28% solution of the sodium salt of sulfated octyl phenoxyethoxyethanol in a mixture of water and ethyl alcohol in the ratio of 80 parts by volume of  $H_2O$  to 20 parts by volume of ethyl alcohol is prepared and to the cotton cloth impregnated and calendered, so that on drying 20% solids are left in the cloth. The cloth is found to be an excellent antifogging cloth.

## Example 2

A solution is formed in a water-isopropyl alcohol mixture containing 85 parts by volume of  $H_2O$  to 15 parts of isopropyl alcohol of 25% of the sulfated sodium salt of octyl phenoxyethoxyethanol and 3% of a monomethyl ether of polyglycol having a melting point of 45° C. The cotton cloth is impregnated and then put through a calender and dried so that 20% solids remain in the cloth.

## Example 3

A solution of an ethyl alcohol-water mixture containing 90 parts by volume of  $H_2O$  to 10 parts by volume of ethyl alcohol is made, containing 5% sodium lauryl sulfate, 20% of the sodium salt of sulfated octyl phenoxyethoxyethanol and 3% of the monomethyl ether of polyglycol having a melting point of 45° C. The cotton cloth is impregnated with this solution. It is put through a calender and allowed to retain sufficient liquid so that on drying 20% of the weight of the cloth is retained. The cloth is an excellent antifogging cloth.

## Example 4

The procedure of Example 1 is followed, excepting that the impregnating solution contains 25% by weight of the sodium salt of sulfated octyl phenoxyethoxyethanol and 3% by weight of the lauric acid ester of a polyethylene glycol having an average molecular weight of 4000.

## Example 5

The procedure of Example 1 is followed excepting that the impregnating solution contains 25% by weight of the sodium salt of sulfated nonyl phenoxyethoxyethanol and 3% by weight of naphthenic acid ester of a polyethylene glycol having an average molecular weight of 4000.

## Example 6

The procedure of Example 1 is followed, excepting that the impregnating solution contains 25% by weight of the sodium salt of sulfated octyl phenoxyethoxyethanol and 3% by weight of the dodecyl monoether of a polyethylene glycol having an average molecular weight of 4000.

## Example 7

The procedure of Example 1 is followed, excepting that the impregnating solution contains 25% by weight of the sodium salt of sulfated octyl phenoxyethoxyethanol and 3% by weight of the nonylphenyl monoether of a polyethylene glycol having an average molecular weight of 4000.

## 4

## Example 8

The procedure of Example 1 is followed, excepting that the impregnating solution contains 14% by weight of the sodium salt of sulfated octyl phenoxyethoxyethanol and 14% by weight of the sodium salt of sulfated nonyl phenoxyethoxyethanol.

By using a more concentrated solution and by allowing more of the solution of the antifogging agent to remain in the fabric before drying the soaked fabric, higher percentages of the antifogging agent may be incorporated.

A method of making a paper impregnated with antifogging material comprises suspending the wood pulp or other cellulose fibres constituting the basic ingredient of the paper, in a solution of the antifogging material having a concentration sufficient to incorporate the desired proportion of antifogging material in the paper, when the paper is formed and dried.

While the invention has been described with particular reference to specific embodiments, it is to be understood that it is not to be limited thereto, but is to be construed broadly and restricted solely by the scope of the appended claims.

## What is claimed is:

1. As an article of manufacture useful in preventing the fogging of glass and the like, comprising a fibrous material having incorporated therein at least 3% by weight based on the original weight of said fibrous material of an alkali metal salt of sulfated alkyl aryloxypolyalkoxy alcohol.
2. The article according to claim 1 wherein said article contains in addition to said alkali metal salt a small quantity of a nonionic wetting agent.
3. The article according to claim 1 wherein said article comprises a mixture of alkali metal salts of sulfated alkyl aryloxypolyalkoxy alcohols.
4. The article according to claim 1 wherein said article contains in addition to said alkali metal salt a small quantity of an alkali metal alkylsulfate anionic wetting agent.
5. A process for impregnating fibrous material in the preparation of an article useful in antifogging of glass and the like, which comprises contacting said fibrous material with a solution containing at least 3% by weight based on the original weight of said fibrous material of an alkali metal salt of a sulfated alkyl aryloxypolyalkoxy alcohol, calendering and drying said fibrous material wherein at least 20% of solids remain in said material and whereby said salt becomes incorporated in said fibrous material.
6. A process according to claim 5 wherein said solution is an aqueous solution.
7. A process according to claim 6 wherein said solution is an aqueous alcoholic solution.
8. A process according to claim 7 wherein the impregnated fibrous material is put through a calender and then dried.
9. An article of manufacture according to claim 1 wherein from 3% to 100% by weight of said alkali metal salt, based on the weight of said fibrous material, is incorporated in the latter.
10. An article of manufacture according to claim 9 wherein said salt is the sodium salt of sulfated octyl phenoxyethoxyethanol.
11. An article of manufacture according to claim 10 having incorporated therein as a secondary wetting agent a monomethyl ether of a polyglycol having a melting point of about 45° C.
12. An article of manufacture according to claim 10 having incorporated therein as a secondary wetting agent a sodium lauryl sulfate and the monomethyl ether of polyglycol having a melting point of 45° C.
13. An article of manufacture according to claim 10 having incorporated therein as a secondary wetting agent the lauric acid ester of a polyethylene glycol having an average molecular weight of 4000.

14. An article of manufacture according to claim 10 having incorporated therein as a secondary wetting agent the dodecyl monoether of a polyethylene glycol having an average molecular weight of 4000.

15. An article of manufacture according to claim 10 having incorporated therein as a secondary wetting agent the nonylphenyl monoether of a polyethylene glycol having an average molecular weight of 4000.

16. An article of manufacture according to claim 9 wherein said salt is a sodium salt of sulfated nonyl phenoxy polyethoxyethanol and having incorporated therein naphthenic acid ester of polyethylene glycol having an average molecular weight of 4000 as a secondary wetting agent.

17. A process according to claim 7 wherein said salt is an alkali metal salt of a sulfated alkyl aryloxypolyalkoxy alcohol.

18. A process according to claim 17 wherein said solution contains at least one secondary wetting agent selected from the group consisting of anionic and non-ionic wetting agents.

19. An article of manufacture according to claim 9 wherein 20% by weight of said alkali metal salt based on the weight of said fibrous material is incorporated in the latter.

References Cited in the file of this patent

UNITED STATES PATENTS

|           |          |               |
|-----------|----------|---------------|
| 1,868,862 | Washburn | July 26, 1932 |
| 2,288,714 | Jones    | July 7, 1942  |
| 2,353,978 | Weber    | July 18, 1944 |
| 2,372,171 | Bennett  | Mar. 27, 1945 |
| 2,489,026 | Gilbert  | Nov. 22, 1949 |
| 2,561,010 | Carson   | July 17, 1951 |

OTHER REFERENCES

Borghetto: "Synthetic Detergents in Textile Processing," Am. Dyestuff Reporter, vol. 37, pp. 112, 113 and 130, Feb. 23, 1948.